

Dec. 21, 1926.

1,611,473

G. W. O. MARTIN

METHOD OF TEMPERING LEATHER, RUBBER, AND COMPOSITION SOLES AND THE LIKE

Filed Feb. 7, 1925



## UNITED STATES PATENT OFFICE.

GILES W. O. MARTIN, OF WEST MEDFORD, MASSACHUSETTS, ASSIGNOR TO AMERICAN SHOE MACHINERY COMPANY, OF EAST BOSTON, MASSACHUSETTS, A CORPORATION OF MASSACHUSETTS.

METHOD OF TEMPERING LEATHER, RUBBER, AND COMPOSITION SOLES AND THE LIKE.

Application filed February 7, 1925. Serial No. 7,670.

My present invention is a novel and improved method of treating certain articles, such for example, as leather, leather soles, crepe rubber soles, composition soles and similar articles for tempering, impregnating and treating the same, and includes a simple, novel and efficient apparatus for carrying out this method.

While my invention is primarily directed to the treating of such articles as leather soles in order to temper the same quickly, expeditiously and to a predetermined extent, yet the process may also be utilized advantageously for other purposes, wherein it is desired to impregnate an article or articles with any desired solution, for preserving, softening, solidifying, coloring or other uses. The invention being directed primarily for treating leather soles by forcing a tempering solution therein, I will describe the same as utilized in its preferred form for this purpose.

It is at present customary in tempering leather, to moisten or "soak" the leather, particularly leather soles, in water or similar liquid, for a considerable time, and then the same are allowed to "mull" sometimes several days in order to permit the soles to become sufficiently moist and to become tempered entirely through for use in subsequent manufacturing processes. Such leather soles are then operated upon in manufacturing boots and shoes, and frequently have to be again tempered, before the numerous processes involved in shoe manufacturing, are completed. It is especially difficult in the case of turn shoes, for example, wherein the leather sole must be in an unusually perfect temper to permit the turning operation without tearing out the stitches and destroying the shoe. Another method of tempering such articles, is that wherein a machine is employed, which both flexes, bends or works the leather, and simultaneously applies a tempering solution, thus effectually working the tempering solution into and through the leather, while also mechanically flexing it. The machine operation just described, is very much quicker than the former method, but some difficulty has been found in the machine tempering method, because of the continual variations

in the amount and degree of moisture or solution which can be applied to successive soles, during the short interval of time in which the sole is passing through the machine. The continual varying texture, density and condition and quality of the leather being operated upon, also presents a difficulty, and resulting in lack of uniformity in both the prior methods of tempering. By my present process I eliminate the difficulties heretofore experienced, and by the application of a predetermined amount of pressure I am enabled to force, quickly, thoroughly and completely, into the leather soles or other articles being treated, any desired amount of solution, tempering compound, coloring solution or treating liquid. This process, therefore, enables the tempering or treating operation, particularly on shoe soles of varying kinds or grades of leather, with a substantially predetermined extent of tempering, as desired, and in an extremely short time, and with the assurance of uniformity in the amount of solution applied to each article, while also insuring the complete penetration of the article being treated by the solution applied thereto. My process contemplates the positive forcing, by pressure appliance, of a solution into an article to be treated, as distinguished from prior tempering and treating methods, wherein the normal capillary attraction of the article was relied upon, or where, as in the said machine operation, a combined working and moisture applying operation was employed.

In carrying out my invention, I have devised an extremely simple, inexpensive, and efficient apparatus, which is much less expensive than any tempering machine of which I am aware, and which apparatus can be of any desired size, power and capacity, and of relatively compact form.

A further object of my present improved apparatus is to provide pressure applying means which can be quickly filled with articles to be tempered, hermetically sealed or substantially so sealed, quickly subjected to the desired pressure, and instantly released after the predetermined time of pressure-applying for the particular articles being treated, has elapsed.

Referring to the drawings, illustrating my

novel apparatus suitable to carry out my improved process of pressure tempering, or treating.

Fig. 1 is a complete diagrammatic view of a suitable apparatus.

Fig. 2 being a cross-sectional view through the pressure applying receptacle.

As shown in the drawings, I have arranged a pressure tank 1, of sufficient capacity to hold a substantial quantity of compressed air, preferably proportional to a repeated transfer from the pressure tank 1 of relatively small quantities to a pressure treating tank 2. The pressure tank 1 is provided with a suitable gauge 3 and release valve 4 and may receive pressure from an air pump 5, through the conduit 6, said air pump being actuated in any desired manner, such as, for example, from a motor 10, and belt 12, actuating the pump 5 from the rotation of the pulley 14 and shaft 15.

With a pressure tank 1 of substantial capacity, the motor 10 and pump 5 can be operated for a sufficient time, until the gauge 25 3 indicates a substantial pressure, say five hundred pounds per square inch. As in the present apparatus I may use a pressure, when operating upon sole leather for tempering, of from thirty pounds to 100 lbs. per 30 square inch, and withdrawing the air necessary for the operation in small quantities from the tank 1; when the pressure tank 1 is thus charged it will supply the apparatus for a considerable period, and for a number of 35 successive treating operations.

My treating tank 2 may be of any suitable size, form, contour and capacity, as herein illustrated being a simple, cylindrical member with a base 20 threaded or secured thereto, and a removable top 21, also threaded thereto. The base 20 carries a bored and tapped recess 22, to receive the pipe 23 and connecting conduit 24 to the pressure tank 1 at 25. A valve 26 controls the release of 40 pressure from the tank 1, and a gauge 27 may be fitted to the conduit 24, to indicate the extent of pressure withdrawn from the tank 1.

At the top 21 is a release valve 30, and attached to the lowest point in the conduit 24 is a valve 31 to permit withdrawal of the liquid or tempering solution from the treating tank 2.

When treating leather soles for tempering, I first remove the cap 21, then fill the receptacle 2 with treating solution, to a sufficient level to more than cover the soles. This solution may be water or any usual leather tempering solution and the same 55 when partially filling the pressure receptacle 2 will also partially fill the conduit 24 up to a similar level therein, which is preferably below the pressure gauge 27. As here indicated, these levels in the tank 2 and pipe 24 60 are indicated at 33 and 34, which levels are

those attained after the bunch of soles designated generally at 35, are placed in the treating tank.

These soles are usually blanks, i. e., cut to blank form with square ends and united 70 around the center portion with a wire or fastening 36. For my pressure treating, this fastening 36 may be left intact, if desired, as the pressure applied is usually sufficient to permeate the entire thickness of the bunch 75 of soles, and to percolate through the interstices between the layers of leather forming the bunch 35. If desired, however, the binder 36 may be cut, in which case the individual leather blanks will fall partially 80 apart, as indicated in dotted lines, Fig. 2, at 37 and 38. In either case a plurality of these articles are fitted within the pressure tank 2, the cap 21 threaded thereon, a tight fit being insured by the use of a spanner if 85 desired, engaging the recesses 39, 39, as indicated, and with the valves 30 and 31 shut. Thereupon the operator manipulates the valve 26 to open the same, permitting a flow of pressure from the tank 1, through the 90 conduit 24 and pipe 23 into the interior of the treating tank 2. The indicator 27 will register the pressure attained, the first action being to force the compressed air against the water level 34 in the conduit 24 downwardly, and either entirely out of the conduit 24, or the air will force thereby into the tank 2 and accumulate in the space above the liquid level 33, thus imparting desired 95 pressure to the liquid or tempering solution, 100 which will simultaneously force the solution into the fibres or pores of the leather blanks 35 and compress or displace the air therein contained, which latter may accumulate in the space above the liquid level 33. As soon 105 as the gauge 27 registers the desired pressure 30 to 100 lbs., for example, the valve 26 is shut off, and this pressure thus attained in the tank 2, is maintained for a few seconds or moments, until the tempering solution 110 is sufficiently forced into the leather blanks to thoroughly temper the same.

While I may vary the pressure in the tank 2 as desired, taking care, however, not to permit a greater pressure in this 115 tank than would injure the fabric, texture or composition of the article being treated, and although greater pressure will insure quicker permeation, yet I believe it ordinarily desirable to supply a relatively slight 120 pressure and proportionately prolong the application. Either method, however, can of course be employed and will be varied for different articles being treated. Furthermore, differing degrees of pressure and periods of time to maintain this pressure, will depend, not only upon the article being so treated, but also upon the solution or treating liquid itself. Thus with a loose composition sole for example, and a relatively 125 130

thick or viscous solution to be applied to same, the amount of pressure and the length of time can be increased or decreased as desired for best results. Furthermore, I may 5 vary the temperature in the treating tank 2 if desired, and may utilize to advantage, for some work, steam in place of compressed air, or of course any other gaseous liquid capable of transmitting pressure from a source of 10 supply to and into the tank 2. As soon as desired lapse of time for the particular work at hand, and allowing for the degree of permeability of the articles being treated and the flow therein of the solution being 15 employed, the valve 30 is released, the pressure on the interior of the tank 2 thus quickly relieved and the cap 21 removed. Thereupon the leather blanks 35 or other articles are withdrawn, a new supply positioned, further solution applied from time to time as 20 desired, and the cap 21 replaced and the operation repeated.

I find that my pressure treating process in the apparatus just described, when utilized 25 on such articles as leather, is of special value, in that the tempering solution is positively forced into the leather, quickly and without other effort, or without disturbing the packages of the leather. In fact, I can thus 30 temper such a compound article as two sole blanks, united or cemented together by waterproof adhesive, through which no other tempering solution could be applied. By my method, I am enabled to positively force the 35 tempering solution into both such sole members of a cemented blank, and to thoroughly impregnate them with the tempering solution, and without disturbing the adhesion or cement, withdrawing the soles from the 40 tank 2 ready for use.

As above explained, I believe that my present method is of distinct novelty, par-

ticularly in forcing solutions, tempering compounds or the like liquids, into more or less solid substances. I find that this method 45 and my apparatus as above described, can be employed for waterproofing materials, utilizing a rubber solution for this purpose if desired. Furthermore, I can use my present method and apparatus to great advantage 50 in treating rubber soles, whether of vulcanized rubber or of crepe or unvulcanized rubber, whether a coating, treating, or solution, either for hardening or softening, is desired. My process and apparatus further 55 more can be readily used where the application of heat is essential to the treatment of the articles, and without any expensive additions or changes.

My invention is further described and defined in the form of claims as follows:

1. The improved method of tempering boot and shoe soles, which consists in immersing the sole to be tempered in a solution of tempering material, enclosing the 65 same in a substantially airtight receptacle, and applying gaseous fluid under pressure for a time sufficient to force the tempering solution into the sole, releasing the pressure and removing the sole.

2. The improved process of tempering boot and shoe soles of leather, composition or the like, which consists in applying a plurality of soles into a pressure receiving receptacle, supplying a quantity of tempering 70 liquid in said receptacle, sealing the receptacle, applying air under pressure thereto, and maintaining said pressure to force the tempering solution into the soles, thereupon 75 releasing the pressure, opening the receptacle 80 and removing the tempered soles.

In testimony whereof, I have signed my name to this specification.

GILES W. O. MARTIN.